

July 5, 1932.

C. DREYFUS ET AL

1,866,153

PARTIAL SAPONIFICATION OF CELLULOSE ESTER MATERIAL

Filed Oct. 22, 1929



INVENTORS  
CAMILLE DREYFUS  
HERBERT PLATT  
BY  
*J. Seltzer and Leiberman*  
ATTORNEYS

## UNITED STATES PATENT OFFICE

CAMILLE DREYFUS, OF NEW YORK, N. Y., AND HERBERT PLATT, OF CUMBERLAND, MARYLAND, ASSIGNORS TO CELANESE CORPORATION OF AMERICA, A CORPORATION OF DELAWARE

## PARTIAL SAPONIFICATION OF CELLULOSE ESTER MATERIAL

Application filed October 22, 1929. Serial No. 401,578.

This invention relates to the treatment of textile material containing organic esters of cellulose, whereby the safe ironing point of the same is improved and other desirable properties are imparted thereto.

5 An object of our invention is to increase the safe ironing point of textile materials containing organic esters of cellulose by the partial saponification of the same in a continuous manner. Other objects of our invention will appear from the following detailed description.

10 The partial saponification of organic esters of cellulose textile material to increase the safe ironing point of the same is attended with many difficulties owing to the fact that unless the same be carried out under certain definite conditions, the saponification proceeds unevenly and level dyeing of the textile material is not possible. Furthermore for 15 reasons of economy, it is desirable to carry out the partial saponification in a continuous manner.

We have found that if an aqueous solution 20 of an alkaline material is applied to a moving fabric containing organic esters of cellulose yarn, and then a weaker alkaline solution is applied, and then the fabric is washed, all operations proceeding continuously, excellent 25 results are obtained. The organic ester of cellulose filaments of the fibre is intensely saponified on the surface thereof in an even manner, with the result that the safe ironing point of the same is raised and the fabric is 30 capable of being dyed level. Moreover, by this process, the fabric is partially saponified and scoured at the same time, thus avoiding the necessity of scouring as a separate 35 operation.

40 In accordance with our invention, we partially saponify fabric containing yarns or filaments of organic esters of cellulose by continuously applying thereto a comparatively strong solution of an alkaline material, then 45 continuously applying a weaker alkaline solution, and then continuously washing with water in a series of washers so as to wash out all the alkaline material and metallic salts formed by the saponification.

50 The fabric to be treated may contain yarns

of any suitable ester of cellulose such as cellulose acetate, cellulose formate, cellulose propionate and cellulose butyrate. The fabric need not consist wholly of organic esters of cellulose but may also contain other fibres such as cotton or reconstituted cellulose.

55 The alkaline material applied in the saponifying solutions may be any suitable one such as sodium hydroxide or potassium hydroxide, which may be replaced in whole or in part by alkaline salts such as the carbonate of sodium or potassium, the silicate of sodium or potassium, or the sulphide of sodium or potassium.

60 As stated the fabric is first treated with an alkaline solution of comparatively greater concentration. This solution is preferably of an alkalinity corresponding to a concentration of 4 to 7% of sodium hydroxide and is preferably at room temperatures. It may be 65 applied to the fabric in any suitable manner such as on a pad, by a jig or in a box.

70 After the stronger alkaline solution has been applied, a weaker alkaline solution is then applied. This alkaline solution is of a 75 concentration corresponding to 2 to 4% of caustic soda and is preferably at a temperature of 70° to 85° C.

80 After the application of the weaker alkaline solution, the fabric is thoroughly washed in water, preferably of a temperature of 70° to 85° C., in a series of washers which may be in the form of boxes, jigs, etc. During the washing, the fabric may be subjected to an intermediate spray of water, and excess 85 water may be expressed from the fabric by means of nips before the same proceeds to the next washing bath.

85 The fabric may be first dyed and then subjected to the partial saponification process, or it may be dyed subsequent to such process.

90 The fabric after having been treated in this manner contains fibres of cellulose esters that are intensely saponified on the surface thereof. The safe ironing point of the fabric 95 is materially increased and the fabric is capable of level dyeing.

In order further to illustrate our invention, reference is had to the accompanying drawing, wherein

Figure 1 is a diagrammatic view of apparatus that may be employed for carrying out one form of our invention, and

Figure 2 is a diagrammatic view of apparatus for carrying out a second form of our invention.

Referring to Figure 1, an example of carrying out this invention will be described.

The fabric 1 consisting wholly of yarns of cellulose acetate is passed from the roll 2 into the jig 3 where it is subjected to an aqueous bath containing from 5 to 6% of caustic soda. The fabric then passes around the rolls 4 to the jig 5 which contains an aqueous solution of 3% caustic soda, which solution is at 80° C. The fabric then proceeds around the roll 6 to the jig 7 which contains water at 80° C. and where it is subjected to its first washing treatment. In passing from the jig 7, the fabric may be subjected to a spray of water issuing from the spray pipe 8, and then passes around the rolls 9 to the washing jig 10 which contains water at 80° C. The fabric may then be subjected to a second spray from pipe 11 and then passes around the rolls 12 to the jig 13 where it is given its final washing with water at 80° C. and is then passed over the roll 14 and then batched, the arrangement being that the rate of travel of the fabric through the baths is substantially uniform. The fabric thus treated is partially saponified and scoured and may then be given any subsequent finishing treatment such as dyeing, printing, etc.

Referring to Figure 2, another example of carrying out our invention will be described. The fabric 1 consisting wholly of cellulose acetate yarn is passed from the roll 20 to the padder 21 which contains a caustic soda solution of 5% concentration at room temperature. The fabric is caused to pass under the surface of the caustic soda solution by means of the roll 22 and then passes between the padding rolls 23 to the compensator 24. The compensator 24 comprises the rolls 25, 26 and 27. The roll 26 is mounted so that it may move vertically in order to take up slack on the fabric 1. From the compensator 24, the fabric passes to the box 28 containing caustic soda solution of 3% concentration at 85° C. From the box 28 the fabric passes between the nip rolls 29 which removes the excess of the caustic soda solution contained on the fabric. The fabric then passes to the first washing box 30 which contains running water at 85° C. and on leaving the same may be subjected to a spray of water issuing from the spray pipe 31. The fabric is then passed between the nip rollers 32 to remove excess of washing water and then passes to the second washing box 33 containing running water at 85° C. On leaving the washing box 33, the fabric may be sprayed with water from spray pipe 34, passed between nip rolls 35, and then rolled up as roll 36. This fabric

has been simultaneously partially saponified and scoured and may be subjected to any finishing treatment desired.

It is to be understood that the foregoing detailed description is given merely by way of illustration, and that many variations may be made therein without departing from the spirit of our invention.

Having described our invention, what we claim and desire to secure by Letters Patent is:

1. Method of partially saponifying fabric containing organic esters of cellulose comprising applying an alkaline solution of relatively greater concentration to the fabric and then applying an alkaline solution of less concentration, the operations being performed while the fabric is moving continuously.

2. Method of partially saponifying fabric containing cellulose acetate comprising applying an alkaline solution of relatively greater concentration to the fabric and then applying an alkaline solution of less concentration, the operations being performed while the fabric is moving continuously.

3. Method of partially saponifying fabric containing organic esters of cellulose comprising applying an alkaline solution of relatively greater concentration to the fabric, then applying an alkaline solution of less concentration, and then washing, the operations being performed while the fabric is moving continuously.

4. Method of partially saponifying fabric containing cellulose acetate comprising applying an alkaline solution of relatively greater concentration to the fabric, then applying an alkaline solution of less concentration, and then washing, the operations being performed while the fabric is moving continuously.

5. Method of partially saponifying fabric containing organic esters of cellulose continuously comprising applying thereto an alkaline solution corresponding to a solution of sodium hydroxide of substantially 4 to 7% concentration, then applying an alkaline solution corresponding to a solution of sodium hydroxide of substantially 2 to 4% concentration and then washing with water, the operations being performed while the fabric is moving continuously.

6. Method of partially saponifying fabric containing cellulose acetate continuously comprising applying thereto an alkaline solution corresponding to a solution of sodium hydroxide of substantially 4 to 7% concentration, then applying an alkaline solution corresponding to a solution of sodium hydroxide of substantially 2 to 4% concentration and then washing with water, the operations being performed while the fabric is moving continuously.

7. Method of partially saponifying fabric

comprising organic esters of cellulose continuously comprising applying thereto an alkaline solution corresponding to a solution of sodium hydroxide of substantially 4 to 7% concentration at substantially room temperatures, then applying an alkaline solution corresponding to a solution of sodium hydroxide of substantially 2 to 4% concentration at substantially 70° to 85° C., and  
10 then washing with water at temperatures of substantially 70 to 85° C., the operations being performed while the fabric is moving continuously.

8. Method of partially saponifying fabric  
15 comprising cellulose acetate continuously comprising applying thereto an alkaline solution corresponding to a solution of sodium hydroxide of substantially 4 to 7% concentration at substantially room temperatures,  
20 then applying an alkaline solution corresponding to a solution of sodium hydroxide of substantially 2 to 4% concentration at substantially 70° to 85° C., and then washing with water at temperatures of substantially  
25 70 to 85° C., the operations being performed while the fabric is moving continuously.

In testimony whereof, we have hereunto  
subscribed our names.

CAMILLE DREYFUS.  
HERBERT PLATT.

35

40

45

50

55

60